

No. 812,810.

PATENTED FEB. 20, 1906.

W. BRINTON.

CAST MANGANESE STEEL RAIL.

APPLICATION FILED MAY 4, 1904.

*Fig. 1.*



2



*Fig. 2.*

Witnesses:

*P.M. Pittman*  
Robert Ait

Inventor:

*Walter Brinton,*  
By his Attorney

*F.H. Richards.*

# UNITED STATES PATENT OFFICE

WALTER BRINTON, OF HIGH BRIDGE, NEW JERSEY, ASSIGNOR TO TAYLOR  
IRON AND STEEL COMPANY, A CORPORATION OF NEW JERSEY.

## CAST MANGANESE-STEEL RAIL.

No. 812,810.

Specification of Letters Patent.

Patented Feb. 20, 1906.

Application filed May 4, 1904. Serial No. 206,800.

*To all whom it may concern:*

Be it known that I, WALTER BRINTON, a citizen of the United States, residing in High Bridge, in the county of Hunterdon and State 5 of New Jersey, have invented certain new and useful Improvements in Cast Manganese-Steel Rails, of which the following is a specification.

The present improvement relates to rail-  
road or street-car rails, the object of the in-  
vention being to produce a cast manganese-  
steel rail.

A further object of the invention is the pro-  
vision of a steel rail adapted for railroad or  
street-car use of superior quality and greater  
longevity than ordinary steel rails, it being  
particularly well adapted for use at those  
points in the railroad or street-car system  
where there is greater attrition or wear—as,  
for instance, at curves—than at other points  
in such system.

In the accompanying drawings, Figure 1 is  
a perspective view of this rail, and Fig. 2 illus-  
trates one method of casting the same.

Steel rails, as ordinarily made, especially  
when located at curves, quickly become  
worn out, so that the life of the rail is com-  
paratively very short. It has, however, been  
found by practical test that rails produced  
from manganese-steel—that is, that steel com-  
posed of iron and a certain percentage of  
manganese—when properly made have much  
longer life than ordinary steel rails.

The object of the present invention, there-  
fore, is to provide a superior manganese-steel  
rail. In accomplishing this object the rail 2  
is cast into the form in which it is to be used.  
The present practice of making steel rails is  
to after the billet or ingot has been cast sub-  
ject it to a rolling process for the purpose of  
shaping it into the form in which it is to be  
used. By casting the rail into the shape into  
which it is to be used it is unnecessary to roll  
or to further treat it other than for the pur-  
pose of toughening it or to grind the tread-  
surface thereof, so that the particles or mole-  
cules of metal are not interfered with and the  
resisting qualities thereof not decreased, as is  
believed to be the case where the rail is  
rolled into shape, as heretofore, since by roll-  
ing the steel is thereby refined, as such roll-  
ing tends to change the crystalline condition  
of the rail into a different or fibrous condition,  
in which condition it is believed it does not re-

sist wear so well as when left in the condition 5  
in which it is when cast. In the present in-  
stance the final form of the rail, or that form  
which, as stated, is the form in which it is to  
be used is obtained by the casting of such  
rail into its final shape without any rolling or 10  
other shaping of such rail, it being subjected  
to no further treatment thereof other than a  
toughening treatment and the finishing of  
the tread-surface of such rail. After the rail  
is cast in the form in which it is to be used, 15  
and in which form it would be extremely brit-  
tle unless toughened, it is subjected to heat  
treatment for the purpose of toughening such  
rail. For this purpose I have found that it  
is desirable in order to prevent the setting 20  
up of dangerous internal and contracting  
strains, which cause cracks in the casting, and  
when the rail after it has been cast has so-  
lidified to that extent which will permit the  
same to be properly handled, or, in other 25  
words, when it has reached that point where  
its strength is sufficient to retain its own  
weight without warping and it is freed from  
any parts of the mold which would have a  
tendency to retard the contraction or shrink- 30  
age which commences very soon after casting,  
to subject it to treatment to prevent a too-  
rapid cooling, and consequently a too-rapid  
shrinkage or contraction thereof, and to main- 35  
tain therein a portion of its original heat de-  
termined by the size and character of the rail.  
In other words, the cooling of the casting is  
checked, so that such casting will retain therein  
a portion of its heat varying according to the 40  
size and character of the casting which I  
have found in practice to range between a  
point about 100°—that is to say, above nor-  
mal atmospheric temperature—and 1,000°  
Fahrenheit, according to the size and shape 45  
of the casting. This checking or the main-  
taining therein of a portion of its original  
heat is accomplished in one way by covering  
the casting with sand or preferably placing  
the same in a pit prepared for that purpose, 50  
from which drafts of air are entirely excluded,  
so that all parts of the casting are kept at a  
uniform temperature throughout until they  
have cooled down to the right degree of heat  
for the final toughening. By means of this 55  
preparatory step by which the rail is prevent-  
ed from becoming cold, or substantially so,  
the metal is never permitted to reach a pe-  
riod of rest from absence of heat, which is be-

lieved to be the cause of intense and dangerous contracting strains before final toughening, and the too-rapid cooling of such rail is prevented, so that a gradual and uniform cooling thereof down to the right degree of heat for the final toughening is maintained. The casting is then subjected to heat treatment by in the present instance placing the same in a furnace the temperature of which corresponds or substantially corresponds to the temperature of the cast rail at the time it is placed in such furnace, it then being preferably rapidly heated up to a predetermined point—say, for instance, substantially an orange-heat—whereupon it is removed and cooled, usually by being immersed quickly in water, such as brine-water, although this step may be effected by other suitable processes. By this means I am able to provide a perfectly solid homogeneous cast manganese-steel rail cast into the shape in which it is to be used without the necessity of rolling or other shaping treatment. The tread is then smoothed or finished by grinding, which is the only practicable way of accomplishing this step, since manganese steel cannot be cut or drilled in any practicable manner.

By actual demonstration rails made in accordance with this process and placed on the elevated roads of Boston, Massachusetts, at curves where the wear is very great outlast sixty of the ordinary steel rails heretofore used, and it has not yet been necessary to replace the rails, so that the test has not been completed.

I claim as my invention—

1. As a new article of manufacture, a manganese-steel rail of regulation size and form produced by casting it in the form in which it is to be used as a completed rail, and then toughening such rail.

2. As a new article of manufacture, a manganese-steel rail produced by casting it in the form in which it is to be used as a completed rail and thereupon toughening the rail by heating it and then cooling it.

3. As a new article of manufacture, a manganese-steel rail produced by casting it in substantially the form in which it is to be

used; thereupon arresting the cooling of the rail after solidification; then toughening the rail by heating it rapidly up to a predetermined temperature, and then cooling it rapidly.

4. As a new article of manufacture, a manganese-steel rail produced by casting it in substantially the form in which it is to be used; thereupon arresting the cooling of the rail after solidification; thereupon placing the rail in a furnace having a temperature substantially corresponding to the then temperature of the rail and rapidly heating the rail in such furnace up to a predetermined temperature and thereupon immersing the rail in a cooling-bath.

5. As a new article of manufacture, a manganese-steel rail produced by casting it in substantially the form in which it is to be used; thereupon arresting the cooling of the rail after solidification; and then toughening the rail by heating it and then cooling it.

6. As a new article of manufacture, a manganese-steel rail produced by casting it in substantially the form in which it is to be used as a completed rail, then checking the cooling of the rail after solidification and before such rail reaches a period of rest from absence of heat, and then heating such rail beginning with the furnace in a heated state and applying the heat until the rail has reached a predetermined temperature, and then plunging the rail in cold water.

7. As a new article of manufacture, a manganese-steel rail produced by casting it in substantially the form in which it is to be used as a completed rail, then checking the cooling of the rail after solidification at a predetermined point above normal atmospheric temperature, then heating such rail beginning with the furnace in a heated state substantially corresponding to the temperature of the rail when the cooling thereof is checked, and then finally cooling the rail.

WALTER BRINTON.

Witnesses:

JACOB STRUBLE,  
PERCIVAL CHRYSTIE.